

## UNITED STATES PATENT OFFICE

HARRY HEY AND ARTHUR FANNIN EVANS, OF MELBOURNE, VICTORIA, AND ROWLAND THOMAS DRYLL WILLIAMS AND ARCHIBALD PHILIP NEWALL, OF RISDON, HOBART, TASMANIA, AUSTRALIA, ASSIGNORS TO ELECTROLYTIC ZINC COMPANY OF AUSTRALASIA LIMITED, OF MELBOURNE, AUSTRALIA

## ELECTROLYTIC RECOVERY OF ZINC

No Drawing. Application filed December 17 1927, Serial No. 240,923, and in Australia December 29, 1926.

This invention relates to certain improvements in the electrolytic recovery of zinc and refers more especially to the electrolysis of zinc sulphate solutions obtained from the 5 leaching of roasted zinc ores with sulphuric acid or spent electrolyte.

In the electrolysis of zinc sulphate solutions as at present practised, it is customary to employ lead anodes and aluminum cathodes and it is usual to add a small amount of 10 glue for the purposes of inhibiting the toxic effect of cobalt and/or other substances present in the solution.

In the electrolysis of zinc sulphate solutions containing say 100 grams per litre of 15 zinc as zinc sulphate and 100 milligrams of cobalt as cobalt sulphate, it has been found necessary to add from 3 to 4 lbs. of glue per ton of cathode zinc produced which is equivalent to from 60 to 70 milligrams of glue per 20 litre of solution passing to the electrolytic cells. Owing to inefficient purification small quantities of toxic elements, such as arsenic and copper, are sometimes present in the electrolyte. Owing to the presence of these toxic 25 substances and possibly other causes the ampere efficiency of the electrolysis is sometimes reduced and the quality of the cathode zinc produced affected.

The object of this invention is to provide certain improvements in the electrolysis of zinc sulphate solutions whereby improved current efficiencies may be obtained.

We have found if the electrolysis of zinc 35 sulphate solutions is carried out in the presence of small amounts of antimony in the electrolyte, such amounts being less than will materially affect the nature of the zinc deposited on the cathodes, improved current 40 efficiencies can be obtained. By small quantities we mean 0.5 milligrams per litre or less.

Consequently this invention comprises the addition to the electrolyte of such quantities of antimony as will ensure improved current 45 efficiencies (such as by counteracting the deleterious effect of toxic compounds) but less than such quantities as will affect the nature or condition of the zinc deposited on the cathodes.

The addition of antimony to the electro-

lyte for the purpose of this invention may be effected either in the form of a soluble salt such as antimony, tartrate, or by the use of anodes containing antimony.

Care must be exercised in seeing that an 55 excessive amount of antimony is not present whether derived from soluble salts of antimony added direct to the electrolyte, or from antimonial lead anodes, as excessive amounts will give a very rough deposit of cathode 60 zinc which yields excessive dross when melted. It is therefore necessary to see that the addition of antimony to the electrolyte is closely controlled.

The quantity of antimony present may be 65 judged by the usual well-known characteristics of the zinc plates on the cathodes and such characteristics will afford a guide to the amount of additions of antimony which may be permitted.

Experiments have shown that with an electrolyte which upon electrolysis produced a spent solution containing from 55 to 65 grams of sulphuric acid per litre, appreciably better 70 ampere efficiencies have been obtained with antimony present to the extent of from 0.1 to .5 milligrams per litre as compared with the same conditions when antimony was absent.

A further advantage arises from the modification of this invention wherein the antimony is added to the electrolyte through the medium of an antimonial lead anode in that the antimony strengthens the anode and renders it less liable to buckling or warping 85 whereby a more even current density may be obtained in the cells increasing the over-all ampere efficiency.

In this connection we have found that anodes composed of an alloy of lead and antimony in which the antimony content is from one half ( $\frac{1}{2}$ ) to one and one half ( $1\frac{1}{2}$ ) per cent give very satisfactory results, having regard to current efficiencies on the one hand and the condition of the cathode zinc deposited on the other.

We claim:

1. In the electrolysis of zinc sulphate solutions, containing a toxic substance of the nature of cobalt, the addition to the electrolyte 100

of a soluble salt of antimony in such quantities as will be less than will materially affect the nature of the zinc deposited on the cathodes but sufficient to counteract the deleterious effect of the said toxic substance.

2. In the electrolytic recovery of zinc, the electrolysis of zinc sulphate solutions, containing a toxic substance of the nature of cobalt, the addition to the electrolyte of a soluble salt of antimony in such quantities as will provide an antimony content in the electrolyte of from about 0.1 to about 0.5 milligrams of antimony per litre.

In witness whereof we hereunto affix our  
15 signatures.

HARRY HEY.

ARTHUR FANNIN EVANS.

ROWLAND THOMAS DRYLL WILLIAMS.

ARCHIBALD PHILIP NEWALL.

20

25

30

35

40

45

50

55

60